

June 28, 1960

J. L. WALKER ET AL

2,943,007

METHOD FOR CASTING AND WORKING GRAIN ORIENTED INGOTS

Filed Aug. 26, 1957

Fig. 1.



Fig. 4.



Fig. 2.



Fig. 3.



Fig. 5.



Inventors:  
John L. Walker;  
Henry J. Fisher,  
by Paul A. Frank  
Their Attorney.

# United States Patent Office

2,943,007

Patented June 28, 1960

1

2,943,007

## METHOD FOR CASTING AND WORKING GRAIN ORIENTED INGOTS

John L. Walter, Scotia, and Henry J. Fisher, Schenectady, N.Y., assignors to General Electric Company, a corporation of New York

Filed Aug. 26, 1957, Ser. No. 680,360

6 Claims. (Cl. 148—2)

This invention relates to "soft" magnetic materials and more particularly to improved grain oriented ingots or castings composed of iron and soft magnetic alloys of iron and silicon, iron and aluminum and iron and molybdenum constituting cast intermediates or blanks from which polycrystalline metal sheet material may be prepared by rolling and appropriate heat treatment to have a high percentage of its grains oriented as "cube texture," to a method of preparing such cast intermediates or blanks and to a method of preparing cube texture sheet material therefrom.

As pointed out in a co-pending application for United States Letters Patent, Ser. No. 610,909 filed September 20, 1956, Walter and Hibbard, of which one of the present applicants is a joint inventor and which is assigned to the assignee of this application and filed concurrently with application Ser. No. 610,907 filed September 20, 1956, now abandoned, of which this application is a continuation-in-part, polycrystalline, magnetically "soft," sheet metal having a high proportion of the grains thereof "singly" oriented with respect to the rolling direction and the plane of the sheet has for some years past been utilized as a saturable core material in electrical and electronic apparatus. These previously known oriented sheet materials have usually been composed principally of iron with about 5% or less silicon and have had the body centered cubic lattice form at temperatures below several hundred degrees centigrade. The preferred orientation of these previously known sheet materials has been characterized by a high proportion of their grains having their body-centered cubic lattice forms oriented such that the so-called (110) planes thereof lie substantially in planes parallel to the plane of the sheet with four of the unit cube edges being substantially parallel to the rolling direction of the sheet. This particular orientation is usually designated as the (110) [001] orientation.

As will be readily recognized by those skilled in the metallurgical arts, the numerical notation of the (110) crystallographic plane previously used is the accepted description of a plane in the unit cube containing diagonally opposite cube edges according to the Miller Crystallographic Index System. Similar numerical designations of crystal structure and directions used hereinafter will be set forth in accordance with the same index system, a more complete discussion of which may be found, for example, in "Structure of Metals" by C. S. Barrett, McGraw-Hill Book Company, Inc., New York, 2nd edition, 1952, pages 1-25.

Sheet metals having this (110) [001] orientation may be otherwise described as an elongated polycrystalline body of sheet metal having the body-centered cubic lattice form produced by conventional rolling procedures in which a majority of the grains of the sheet have their crystal structure so related to the direction of rolling and the plane of the sheet that the body-centered unit cube lattices thereof are "standing on edge" with respect to the plane of the sheet and each unit cube has two

2

opposite cube faces perpendicular to the direction of rolling and the plane of the sheet. This orientation is more completely described in the previously mentioned co-pending application wherein such materials are described as "singly oriented" and which additionally discloses that since the direction of easiest magnetization in these materials is along the cube edges of the unit cube lattice form, these previously known singly oriented sheet materials have had less desirable magnetic properties in the transverse to rolling direction compared to the same properties in the rolling direction.

In the previously referenced patent application, it is disclosed that polycrystalline, rolled, body-centered cubic, soft magnetic sheet material having improved magnetic properties may be prepared by properly rolling and heat treating a grain oriented cast intermediate or blank. The improved polycrystalline sheet material so produced is characterized as having a majority of the grains of the sheet oriented in a "cube texture." This cube texture may be described as an (100) [001] orientation. Stated otherwise, a high proportion of the grains of such cube texture material have their crystal lattices oriented so that two opposite faces of the unit cube are parallel to the rolling plane of the sheet, two other opposite cube faces are perpendicular to the rolling plane and parallel to the rolling direction and the two remaining cube faces are perpendicular to the rolling plane and perpendicular to the rolling direction. Sheet materials consisting essentially of iron, iron and up to about 5% silicon, iron and up to about 8% aluminum, and iron and up to about 5% molybdenum, having this orientation have been found to have greatly improved magnetic properties, particularly in the transverse to rolling direction, compared to previously known polycrystalline oriented sheet materials of comparable compositions. It was found, however, that in order to realize these beneficial results in a final sheet metal product that the grain oriented casting then employed must be rolled in either one or the other of two relatively restricted modes.

As disclosed in the previously referenced application, molten metal consisting principally of iron is cast into an ingot consisting essentially of a plurality of elongated columnar grains whose longitudinal axes are substantially parallel to each other. The improved magnetic sheet material previously referred to may then be prepared by appropriately rolling and heat treating such an ingot or a portion thereof. In order to produce the desired cube texture in the finished sheet or strip material, it has been found desirable to confine the majority of the rolling passes by which the material is worked to a direction in which the longitudinal axes of the elongated columnar grains of the casting are maintained substantially perpendicular to an imaginary line lying between the working rolls which is substantially mutually parallel to the axis of rotation of each of the rolls. As more particularly disclosed in the previously referenced application, this direction of the longitudinal axes of the columnar grains in the casting may be selected from one or the other of two general relationships of the direction with respect to the working or rolling plane and the rolling direction. For example, the direction in the casting most nearly parallel to all the longitudinal axes of the elongated columnar grains thereof, must be maintained substantially parallel to the rolling plane and to the rolling direction during a majority of the reducing rolling passes and the longitudinal axes of a majority of the elongated grains should not deviate more than about 20 degrees from this parallelism. In the other preferred alternative relationship, the direction in the casting most nearly parallel to all longitudinal axes of the elongated columnar grains thereof must be maintained substantially perpendicular to the rolling plane.

and to the rolling direction during a majority of the reducing rolling passes, and the longitudinal axes of a majority of the elongated grains should not deviate more than about 20 degrees from this perpendicular relationship. It has been found that if the reduction of the casting to sheet metal by rolling is accomplished by maintaining the direction in the casting most nearly parallel to the longitudinal axes of the columnar grains substantially parallel to the rolling plane and substantially perpendicular to the rolling direction during a majority of the reducing rolling passes, the resulting annealed sheet metal does not have the well-developed cube texture characteristic of materials produced by the other two previously disclosed modes of working and consequently does not have the desirable magnetic properties of the materials produced by these other two modes of rolling.

In such grain oriented castings, it has been found that the body-centered cubic lattices of each of the elongated columnar grains are similarly oriented with respect to the longitudinal axis of each elongated grain in that certain cube faces of the lattices in each grain are arranged substantially perpendicular to the longitudinal axis of that elongated grain. However, with respect to different elongated grains which have their longitudinal axes substantially parallel, the cube faces of one grain's lattice which are substantially parallel to that grain's longitudinal axis are only occasionally parallel to corresponding cube faces in other elongated grains.

It would be desirable to improve the orientation of the elongated columnar grains in the previously described ingots so that a greater number of the grains thereof would have their axes more nearly parallel and thereby reduce the average or net angular deviation of these axes from either of the above noted preferred rolling relationships so that the finished polycrystalline sheet material produced therefrom would have a greater proportion of its constituent grains oriented in the "cube texture." Furthermore, yet further improvements in the cube texture of such sheet or strip material may be achieved if the cubic lattices of the elongated grains of such castings are oriented with respect to each other so that not only are the cube faces which are substantially perpendicular to the longitudinal grain axis in one grain substantially parallel to corresponding cube faces in substantially all other grains, but the other cube faces which are substantially parallel to the longitudinal axis of one elongated grain are substantially parallel to corresponding cube faces in substantially every other elongated grain in the casting. Additionally, by using such an improved grain oriented casting, greater flexibility in rolling limitations may be achieved. For example, such an ingot may be rolled to form sheet metal having well-developed cube texture by "cross-rolling," i.e., by maintaining the direction in the casting most nearly parallel to all the longitudinal axes of the elongated columnar grains substantially parallel to the rolling plane and substantially perpendicular to the rolling direction during a majority of the reducing rolling passes.

Accordingly, it is a principal object of our invention to provide an oriented cast intermediate or blank having an improved, more regular, as-cast macrostructure.

A further object of our invention is the provision of a method whereby such an improved oriented cast intermediate or blank may be prepared.

A yet further object of our invention is the provision of a method whereby such an improved cast intermediate or blank may be reduced by rolling and heat treatment to form sheet material having a well-developed cube texture.

Other and specifically different objects of our invention will become apparent during the course of the detailed disclosure and description which follows.

Briefly stated, in accordance with one aspect of our invention, we provide an improved polycrystalline grain oriented casting constituting an intermediate or blank for subsequent rolling operations, the grain structure of which is principally composed of elongated columnar grains whose longitudinal axes are nearly parallel to each other, the casting being composed principally of iron and having the body-centered cubic lattice form at temperatures below several hundred degrees centigrade, the casting being further characterized by the crystallographic orientation of each individual, elongated, columnar as-cast grain being substantially identically oriented with respect to every other individual elongated columnar as-cast grain in the casting, a method for producing such a casting by pouring molten metal to be cast upon a grain oriented seed of similar chemical composition and by causing the molten metal to solidify in a temperature controlled manner upon such seed, and a method for rolling and heat treating such a casting to produce sheet material therefrom having a well-developed cube texture.

Our invention will be better understood from the following description taken in connection with the accompanying drawings and its scope fully pointed out in the appended claims.

Fig. 1 is a perspective view of a casting composed of columnar as-cast grains, with parts broken away;

Fig. 2 is a sectional view of a portion of the casting of Fig. 1 taken along line 2-2 thereof;

Fig. 3 is a vertical sectional view of a casting apparatus including an ingot cast therein, illustrating one embodiment of our invention;

Fig. 4 is an enlarged view of a portion of the ingot shown in Fig. 3; and

Fig. 5 is a sectional view of the portion of the ingot illustrated in Fig. 4 taken along line 5-5.

As disclosed in the previously referenced application, the cast intermediates or blanks disclosed therein may be prepared according to one aspect of that invention by casting molten metal consisting principally of iron into an elongated tubular mold having preheated side-walls and a cooled bottom. The superheat and the latent heat of the molten metal is substantially all extracted through the cooled bottom of the mold in a continuous manner during solidification of the molten metal causing the solidification to initiate and progress from the cooled bottom of the mold toward the top of the casting. In this manner a casting is produced consisting essentially of a plurality of elongated columnar grains whose longitudinal axes are substantially parallel and which extend in a direction substantially parallel to the direction of solidification of the ingot. This type of casting may be referred to as a "singly" oriented casting in order to more clearly distinguish it from the "doubly" oriented casting of our present invention, the distinguishing structural characteristics of which will be subsequently disclosed.

A portion 10 of such a "singly" oriented casting is schematically shown in perspective in Fig. 1 with parts broken away for greater clarity and with the grain structure of a portion of the casting schematically indicated. While the portion 10 of the singly oriented casting has been shown as a generally rectangular prismatic body, it will be appreciated that this particular form has been arbitrarily selected only for purposes of illustration. As may be seen in the figure, the grain structure of this casting is composed of elongated columnar grains whose longitudinal axes extend in a generally vertical direction as shown. If a slab 11 is prepared from portion 10 by cutting along lines 12 and 13 and along lines 14 and 15 and the slab 11 sectioned along a plane 2-2, for example, the grain structure of the sectioned slab 11 will appear as shown in Figure 2.

In Fig. 2 a portion of such a slab section is shown in which the several irregular areas represent individual columnar grains of the casting sectioned approximately

perpendicular to the longitudinal axes of the several elongated grains. As previously stated, the materials with which our invention is concerned, have the body-centered cubic lattice form at temperatures below several hundred degrees centigrade. Upon examination of these individual grains in representative castings by means of X-ray diffraction techniques, it was found that these individual elongated columnar grains were similarly oriented with respect to their crystal structure, i.e., that the cubic lattice form of each elongated grain was oriented so that certain of the (100) crystallographic planes, which correspond to the planes of the cube faces, are substantially perpendicular to the longitudinal axis of each grain. It was also found, however, that the planes corresponding to the unit cube faces of the crystal lattices of each grain which were necessarily substantially parallel to the longitudinal axis of that grain were only occasionally parallel to similar crystal planes in the other elongated grains. This may be better understood by reference to Fig. 2 in which the previously described grains are schematically illustrated in cross section with respect to the longitudinal axes of said grains and the cube faces schematically shown by the small squares in each grain area indicate the described crystallographic orientation of each grain. It will therefore be seen that each grain in Fig. 2 has its crystal structure oriented so that certain of the crystal planes corresponding to unit cube faces are substantially parallel to the plane of the paper which is substantially perpendicular to the longitudinal axis of each grain. Further, it will be noted in this illustration that only two of the illustrated grains 16 and 17 are substantially identically oriented in all respects, that is, all the planes corresponding to unit cube faces in grain 16 are substantially parallel to corresponding unit cube faces in grain 17. While for purposes of illustration, two grains out of seven are shown having this parallel orientation, no particular significance should be attached to this ratio since no particular ratio has been found or established for this type of parallelism, however, it should be noted that this parallel orientation is found only among a minority of the grains in any particular section of such a casting.

According to one aspect of our invention, however, such a slab may be advantageously utilized to produce a casting consisting essentially of a plurality of elongated grains having a high degree of parallelism. Stated otherwise, such a casting consists essentially of a plurality of elongated columnar grains, the longitudinal axes of substantially all of such columnar grains being substantially parallel to each other and the orientation of the lattice form of each such grain having certain crystallographic planes corresponding to unit cube faces perpendicular to the longitudinal axis of the grain, the remaining unit cube faces being substantially parallel to corresponding cube faces in substantially every other such grain in the casting. Castings made according to our invention having this gross grain structure, may be referred to as being "doubly" oriented.

More specifically, according to our invention, a casting apparatus similar to that disclosed in the previously referenced application may be used to produce a "singly" oriented casting as also set forth in said application. A slab 11 as shown in Figs. 1 and 2 is cut therefrom.

The casting apparatus previously referred to may then be reassembled as it was for casting the single oriented casting. Referring to Fig. 3, this apparatus is schematically illustrated therein and consists of a tubular mold 20 of a refractory material such as fused  $Al_2O_3$ , for example, having open ends. The interior of the mold 20 may have any desired cross-sectional configuration such as circular or rectangular or the like. The bottom end of the mold cavity is closed by the upper surface of a heat extraction member 21 which is preferably constructed of a material having good heat exchange properties such as copper, for example. Member 21 is provided with means for permitting a cooling medium to be circulated in heat

exchange relationship for the extraction of heat from said member. As shown, this may be accomplished, for example, by making heat extraction member 21 in the form of a hollow body and providing pipes 22 and 23 for circulation of a cooling medium such as cold water therethrough.

The tubular mold 20 and the heat extraction member 21 are assembled together as illustrated in Fig. 3 and cooling water is circulated through said member 21 by means of pipes 22 and 23. The interior of the mold cavity is heated to a temperature of about 1400° C. by any convenient means such as, for example, a removable electrical resistance heater while the upper surface of member 21 is maintained at about room temperature or about 20° C. by means of the coolant. Slab 11, which is of sufficient size and configuration to readily lie flatly in the bottom of mold 20 may be preheated if desired to about 1300° C. When the mold sidewalls have been preheated to about 1400° C., the heating means is removed, the preheated slab 11 placed in the bottom of the mold 20 upon surface 21 with a surface presented to the mold cavity consisting of columnar grains sectioned substantially parallel to their longitudinal axes. Molten metal of substantially the same composition as slab 11 is poured into the mold covering slab 11 and substantially filling the mold cavity before the preheated slab can be cooled to any substantial degree by the heat extraction member 21. Coolant is circulated through member 21 until the casting solidifies. During solidification substantially all the superheat and the latent heat from molten metal is continuously extracted through the slab 11 by the heat extraction member 21 and only a small amount of the total heat of the metal is lost through the mold sidewalls and to the atmosphere at the top of the mold. In this manner the heat extraction is substantially entirely unidirectional toward the member 21 and during solidification a temperature gradient is maintained in the metal from top to bottom.

A schematic representation of a vertical cross-section of an ingot 25 produced in this manner is shown in the mold in Fig. 3 after solidification is completed. The seed slab 11 is shown at the bottom of the ingot 25, the location of the former upper surface of such seed slab being shown by dashed line 14. As shown, the bulk of the ingot above the seed slab 11 is composed of a relatively few large columnar grains extending from the seed slab to a zone 26 at the top of the ingot which is comprised of relatively small equiaxed grains of conventional size and configuration. In the interest of clarity these equiaxed grains have not been shown in detail since they are quite conventional in configuration and in practice, are removed along with the "pipe" 27 by shearing or the like from the ingot as scrap.

Upon X-ray examination of the long columnar grains formed between zone 26 and the slab 11 and comprising the bulk of the casting, it will be found that they have their origin in grains of the seed slab 11 which are oriented so as to have a cube face almost nearly parallel to the face of the slab which was exposed to the molten metal and therefore the crystal orientation of these grain bears a substantially parallel relationship to each other. The grains which grow upon solidification from the surface of the seed slab 11 under these conditions assume and continue their growth with substantially the same orientation as the parent grain provided the molten metal poured upon the seed slab 11 melts or tends to melt the surface of the seed slab with which it is in contact before solidification begins. The grains which grow from seed grains having a less favorable orientation do not attain the size of grains which grow from seed grains such as 16 and 17, for example, and tend to be "pinched off," as shown.

In Fig. 4, an enlarged view of the seed slab 11 and metal cast thereon is shown. For purposes of illustration, the seed slab portion shown in Fig. 2 has been reproduced

therein. The upper surface 14 of seed slab 11 is shown as a dashed line to indicate the original dimension of the slab and grains 16 and 17 are similarly reproduced. Dash-dot line 30 represents schematically the degree of melt back of slab 11 by the molten metal before solidification began. The grain structure above line 30 is a result of molten metal which has solidified under the temperature gradient caused by the unidirectional extraction of heat therefrom by member 21. Grains 16' and 17' have substantially the same crystal orientation as grain 16 and 17 from which they grew and grow to the ultimate exclusion of less favorably oriented grains adjacent to or surrounding them and form the larger columnar grains shown in Fig. 3. These larger grains, such as 16' and 17', for example, have substantially completely parallel orientation as shown in Fig. 5, a section taken along 5-5 of Fig. 4. Obviously all the larger columnar grains constituting the body of castings such as casting 25 are similarly oriented and therefore such a casting may be said to be doubly oriented.

In practice, zone 26 and the seed slab 11 and the short, misoriented grains adjacent the seed slab may be removed as scrap leaving a doubly oriented cast intermediate or blank which may then be reduced to cube texture soft magnetic sheet material by appropriate rolling and heat treatment. The polycrystalline sheet material so produced from the doubly oriented cast intermediate made according to our invention has a higher proportion of their grains oriented in the desired cube texture and the limited directional relationships required for processing of the singly oriented cast intermediates are materially increased making the production of such cube texture sheet material substantially easier.

More specifically, and by way of example, an alloy composed of about 3% silicon, about 0.04% carbon, and the balance substantially all iron was melted and cast into a tubular mold of fused  $\text{Al}_2\text{O}_3$  supported upon a water-cooled copper block constituting the bottom closure thereof, as shown, for example in Fig. 3 at 20 and 21 respectively. It should be noted however, that the molten alloy was poured directly upon the copper bottom and that in this casting operation no seed slab 11 was used. The interior side walls of the mold were heated to a temperature of about 1200° to 1400° C. just prior to pouring and, by virtue of the water-cooling, the temperature of the copper bottom was maintained at about 20° C. during the casting and solidification of the ingot. The ingot was sectioned from top to bottom and found to be substantially completely comprised of elongated columnar grains having their axes extending substantially parallel to the longitudinal axis of the ingot or stated otherwise, substantially perpendicular to the copper bottom, with a relatively small zone of equiaxed grains adjacent the upper portion of the ingot which included a small "pipe." The equiaxed grain zone and pipe were removed and a rectangular prism-shaped slab was removed from one half of the sectioned ingot to form a body similar to body 11 of Fig. 1, which was then trimmed to a dimension and configuration compatible with the mold 20 to form a seed slab.

The seed slab thus prepared was heated to about 1300° C. and supported upon the water-cooled copper member 21 within the lower end of a tubular fused  $\text{Al}_2\text{O}_3$  mold 20 with face 14 presented to the mold cavity, the interior side walls of the mold being heated to about 1200° to 1400° C. just prior to casting. A molten alloy composed of about 3 percent silicon, .04 percent carbon, and the balance substantially all iron was cast thereinto, all as previously disclosed and described with reference to Fig. 3. The casting thus produced was vertically sectioned and found to be principally composed of elongated columnar grains 25 extending upwardly from the seed slab 11 and having a relatively small equiaxed zone 26 containing a pipe 27 substantially as illustrated in Fig. 3.

A rectangular prismatic slab 0.300 inch thick was pre-

pared from said sectioned ingot in which a direction substantially parallel to the longitudinal axes of all the elongated columnar grains was substantially parallel to the slab faces and the portions containing the equiaxed grains and pipe and the seed was removed. The slab was then divided approximately into two substantially equal-sized portions each 0.300 inch thick by cutting along a plane perpendicular to the slab faces and the longitudinal axes of the columnar grains. These substantially identical slabs and the sheet material rolled therefrom will be hereinafter designated as "A" and "B" for convenience.

Both slabs A and B were heated to about 1000° C. and reduced in 8 rolling passes to 0.083 inch thick sheet metal without reheating. The hot-rolled strips were reduced at a temperature of about 400° C. to about 0.025 inch thick sheet or strip in a plurality of rolling passes. This strip or sheet material was then annealed by heating in a dry hydrogen atmosphere to a temperature of 1000° C., held for 4 hours and permitted to rapidly cool in the hydrogen atmosphere.

The strips were then cold-reduced by unidirectional rolling to 0.012 inch thick in a plurality of rolling passes. Torque test specimens comprising circular disks 1 inch in diameter were stamped from the strips and annealed in dry hydrogen by heating at about 100° C. per hour to 1200° C., held at that temperature for 5 minutes and slowly cooled, i.e. at about 100° C. per hour.

All the rolling was unidirectional, the A slab being reduced by a rolling schedule during which the direction in the slab substantially parallel to the longitudinal axes of the columnar grains was maintained substantially parallel to the rolling plane and substantially perpendicular to the rolling direction, while the same direction in slab B was maintained substantially parallel to both the rolling direction and the rolling plane.

Conventional torque tests performed in a unidirectional magnetic field of 1,000 oersteds on 16 samples from slab A exhibited an average torque of 97,500 ergs/cc. with average peak ratios of 0.72. Based upon these results, this material has about 79% of its constituent grains oriented in the cube texture. Substantially identically processed sheet material having substantially the same composition obtained from non-seeded columnar ingots rolled with the longitudinal axes of the columnar grains maintained substantially parallel to the rolling plane and perpendicular to the rolling direction during rolling (i.e. cross-rolled) exhibited an average torque of 67,000 ergs/cc., and a peak ratio of about 0.71 for 86 samples. This material has about 54% cube texture.

The material rolled from slab B had an average torque of 109,600 ergs/cc., a peak ratio of 0.75 and therefore was about 89% cube texture.

From the foregoing, it is apparent that a sharp cube texture is obtainable from a seeded columnar ingot when rolled with the direction in the ingot which is nearest to parallel to the longitudinal columnar grains maintained substantially parallel to the rolling plane and perpendicular to the rolling direction, whereas similarly rolling a non-seeded columnar casting produces strip having a much poorer texture. It should be noted that the terms "substantially parallel" and "substantially perpendicular" include directions within 20° of absolute parallel and perpendicular.

It will also be appreciated by those skilled in the art that the oriented seed slab may be composed of an alloy or metal differing in composition from the melt provided it has a melting point substantially the same as the melt, in order to permit melt-back, and a lattice parameter similar to the molten metal so that oriented nucleation and growth of grains having the same orientation as the grains of the seed may be accomplished.

From the foregoing, it will be apparent to those skilled in the art that such seed slabs having higher proportions of grains oriented with respect to the surface presented to the molten metal similar to grains 16 and 17 in Figs.

2 and 3 would be more desirable. Defined in a more general way, the reduction of the casting into sheet metal in accordance with this invention will be carried out by heating the casting to a temperature of from about 700° C. to about 1100° C. and then rolling the heated casting to effect at least a 70% reduction in its thickness. It is then annealed in a hydrogen atmosphere for from 4 hours at about 1000° C. to about 1/2 hour at about 1200° C., cooled and cold rolled (i.e., at room temperature) to a thickness reduction of at least 40%. The resulting cold rolled sheet metal is next annealed and recrystallized by heating to at least 1150° C. in a hydrogen atmosphere and finally slowly cooled in a hydrogen atmosphere.

In view of the foregoing disclosure, it will be apparent to those skilled in the metallurgical arts that we have invented a process whereby the grain orientation of cast ingots of body-centered cubic iron alloys such as alloys containing up to about 5% silicon, balance substantially all iron, up to about 5% molybdenum, balance substantially all iron, and up to about 8% aluminum, balance substantially all iron may be substantially improved.

What we claimed as new and desire to secure by Letters Patent of the United States is:

1. A method for preparing cube texture soft magnetic sheet metal comprising the steps of providing a casting consisting essentially of iron comprising a plurality of elongated columnar grains having their longitudinal axes extending substantially parallel to a first single direction, a majority of said elongated grains having a unit cube face of their crystal lattices substantially parallel to said first direction and substantially perpendicular to a single second direction which is substantially perpendicular to said first direction; reducing the casting into sheet metal by a plurality of rolling passes in the majority of which rolling passes the first direction is maintained substantially parallel to the rolling plane and substantially perpendicular to the rolling direction and the second direction is maintained substantially perpendicular to the rolling plane and to the rolling direction; and annealing the cold rolled sheet metal by heating to at least 1150° C. in a hydrogen atmosphere and slowly cooling the recrystallized sheet metal in the hydrogen atmosphere.

2. The method recited in claim 1 in which the casting is prepared by melting the metal to be cast, bringing the molten metal into contact with a surface of a non-molten body of metal having the body-centered cubic crystal lattice form, said non-molten body being comprised of a plurality of elongated columnar grains having their longitudinal axes extending substantially parallel to a single direction substantially parallel to said surface, maintaining said molten metal in contact with said surface for a period of time sufficient to melt a portion of said surface and withdrawing heat from the molten metal through the seed slab in a direction substantially perpendicular to the surface of the seed slab and thereby solidifying the 55 molten metal on said surface to form an ingot.

3. The method recited in claim 2 in which the casting is prepared by pouring said molten metal into an ingot mold and maintaining a temperature gradient along a single lateral direction of the ingot mold so that substantially all of the grains in the ingot grow during solidification of the metal as elongated columnar grains having their longitudinal axes substantially parallel to the gradient and substantially perpendicular to the surface of the non-molten body of metal.

10 4. The method recited in claim 1 in which the casting is reduced into sheet metal by the steps comprising heating the casting to a temperature of from about 700° to about 1100° C., rolling the heated casting to effect at least a 70% reduction in thickness, annealing in a hydrogen atmosphere for from 4 hours at about 1000° C. to about one-half hour at about 1200° C., cooling the rolled, annealed metal, reducing the thickness of the annealed metal at least 40 percent by cold rolling, annealing the cold rolled sheet metal by heating to at least 1150° C. in a hydrogen atmosphere and slowly cooling the recrystallized sheet metal in the hydrogen atmosphere.

5. A method for casting grain-oriented ingots of magnetic metal consisting essentially of iron comprising the steps of melting the metal to be cast, bringing the molten metal into contact with a surface of a non-molten body of metal consisting essentially of iron, said non-molten body being comprised of a plurality of elongated columnar grains having their longitudinal axes extending substantially parallel to a single direction substantially parallel to said surface, maintaining said molten metal in contact with said surface for a period of time sufficient to melt a portion of said surface and solidifying the molten metal on said surface to form an ingot.

35 6. A method for casting grain-oriented ingots comprising the steps of pouring a molten magnetic metal consisting essentially of iron upon a surface of a body of solid metal consisting essentially of iron, said body of solid metal being comprised of a plurality of elongated columnar grains having their longitudinal axes extending substantially parallel to a single direction substantially parallel to said surface, permitting the surface of said body to become molten and then causing the molten metal to solidify by extracting substantially all the superheat and the latent heat of the molten metal through said body of solid metal.

#### References Cited in the file of this patent

#### UNITED STATES PATENTS

|           |             |               |
|-----------|-------------|---------------|
| 1,793,672 | Bridgman    | Feb. 24, 1931 |
| 1,961,399 | Snook       | June 5, 1934  |
| 2,112,084 | Frey et al. | Mar. 22, 1938 |
| 2,113,537 | Hiemenz     | Apr. 5, 1938  |
| 2,307,391 | Cole et al. | Jan. 5, 1943  |

UNITED STATES PATENT OFFICE  
CERTIFICATE OF CORRECTION

Patent No. 2,943,007

June 28, 1960

John L. Walter et al.

It is hereby certified that error appears in the above numbered patent requiring correction and that the said Letters Patent should read as corrected below.

In the heading to the drawings, name of inventor, for "J. L. WALKER ET AL" read -- J. L. WALTER ET AL --.

Signed and sealed this 20th day of December 1960.

(SEAL)

Attest:

KARL H. AXLINE  
Attesting Officer

ROBERT C. WATSON  
Commissioner of Patents